

June 22, 1926.

1,590,045

C. F. LORENZ

HIGH RESISTANCE ELECTRICAL CONDUCTOR

Filed March 17, 1923

FIG. 1



FIG. 2



FIG. 3



INVENTOR  
CHARLES F. LORENZ  
BY  
*J. F. Lorenz*  
ATTORNEY

## UNITED STATES PATENT OFFICE.

CHARLES FREDERICK LORENZ, OF EAST ORANGE, NEW JERSEY, ASSIGNOR TO WESTINGHOUSE LAMP COMPANY, A CORPORATION OF PENNSYLVANIA.

## HIGH-RESISTANCE ELECTRICAL CONDUCTOR.

Application filed March 17, 1923. Serial No. 625,777.

This invention relates to high resistance electrical conductors and to a method of making the same.

An object of the invention is to provide a conductor of such form as to be of relatively high resistance and which will occupy a comparatively small space.

Another object of the invention is to provide a resistor which will be of a durable character and not readily subject to mechanical injury.

Another object is to provide a resistor that will not be readily over heated.

A further object is to provide a reliable resistor free from the influence of temperature changes.

Other objects and advantages will be apparent upon a reading of the following description.

In making high-resistance conductors, the resistance of which is rated in megohms, various expedients have been resorted to, among which are the deposit of conducting material on a given non-conducting surface in the form of a thin film or of a narrow band. Resistors made by such method may be employed with certain electrical apparatus but resistors of the above type lack the durability desirable in devices of this character.

According to the present invention, a resistor of minute cross sectional area may be produced by providing a cylinder or a tube of an oxide or chemical substance, preferably a refractory oxide, and then applying a streak or winding around the oxide of a material capable of reducing the oxide when both the reducing material and the oxide are heated, in a suitable environment, to a temperature below the melting point of either.

The heating may be accomplished either by the passage of an electric current through the reducing material or by placing the whole in an oven or furnace; the heating being performed in a vacuum or suitable atmosphere. A streak of metal will then be formed upon the oxide owing to the action of the reducing material.

An electrical connection may be made with the metallic streak or thread of metal in any suitable manner and a resistor obtained for various purposes as, for instance, for use as a grid leak in connection with radio apparatus.

A more clear understanding of my invention may be had by reference to the following description and accompanying drawings in which:

Fig. 1 is an elevational view of an oxide body for supporting the resistor;

Fig. 2 is a view of the body as is shown in Fig. 1 but showing a helix thereon of a material capable of reducing the oxide; and,

Fig. 3 shows a complete device ready for use as a resistor.

The invention may be practiced by employing a supporting body in the form of a cylinder or tube 5, preferably of a refractory oxide. A filamentary body, such as a strip or wire 6, may then be wound about the body 5, preferably in the form of a helix. The wire 6 may be of a material capable of reducing the oxide when both are heated to a temperature below the melting point of either.

If desirable, the reducing material may be painted upon the body or it may be applied by abrasion in the form of a pencil mark.

The heating may be accomplished by passing an electrical current through the strip or by placing the body, with the strip thereon, in an oven or furnace, in which they may be heated in a suitable gas inert with respect to the oxide or in a vacuum. A streak of metal 7 of helical formation will then be formed in or about the surface of the oxide, owing to the action of the material of the positioned wire. The body may then be removed from the furnace and the wire discarded. Suitable caps 8 and 9 of a conductive material may be fitted to the ends of the body 5 in such manner that the terminals of the thread or streak 7 will be disposed in contact with the caps. The body may then be varnished for protection from the atmosphere or it may be enclosed in a sealed tube, such as the glass tube 10 shown in Fig. 3, which may be evacuated, or may contain an inert gas.

If desired, the strip 6 may have its ends slightly enlarged to give a greater surface area of conductive material at the points of contact between the caps or conductors 8 and 9. It may, however, be preferable to connect the ends of the wire 5 to cups of a similar material which may fit over the ends of the body 6, thus, when the body is subjected to the reducing action, the layer of

metal upon the body will be connected to a relatively large cylindrical surface at each end to facilitate connection to leads.

A resistor produced by the present method has considerable advantages over resistor elements produced by other methods, particularly those which cause a deposit of a conductive material upon the surface of another body. Such deposited conductors as 10 were heretofore provided required careful handling and were liable to the detrimental effects caused by mechanical abrasion which would result in portions of the resistance material being removed. Such loss of resistance material would obviously seriously affect the value of the element for the purpose for which it was intended.

It will be appreciated that various oxides 20 may be used for the body 6 of the present invention and that different materials may be employed for the helix. As an example, thoria may be chosen as the oxide, in which case, carbon will be a suitable material for the helix. The employment of these two 25 materials may require heating to a temperature something approaching 1400° C. but a considerably higher temperature may be used. The advantage of a resistor produced by the present method consists in the 30 durability thereof, which is evident, since the metal used for the high-resistance resistor will be firmly embedded in, and intimately associated with, the supporting body or the oxide. This fact makes it extremely durable and not readily subject to 35 mechanical injury.

It will be obvious that an oxide, such as 40 chromium or cobalt oxide, may be used as a supporting body or base. A mixture of oxides or other chemical compounds may be employed so that the reduction will give an alloy which has a high-resistance property.

By reason of the close association of the 45 resistor with the mass of oxide or supporting material, the heat-transfer rate may be more rapid and the resistor will not be readily overheated. Furthermore, the resistor will be more reliable in that it will not be readily subject to temperature 50 changes by reason of its intimate contact with the oxide support which facilitates the distribution of heat. As a device for use in connection with radio equipment, the resistor may be of special advantage since it 55 may prove to be free from microphonic effects which are a source of annoyance in resistors heretofore used.

Although the present description and 60 drawings set forth one mode of practicing the invention, it is obvious that modifications may be made therein, for instance, other oxides or suitable chemical compounds capable of reduction may be used for the supporting body and other materials 65 may be used for helix, or the body may be of

a different shape. It is to be understood that such modifications are considered to lie within the spirit and scope of the appended claims.

What is claimed is:

1. A high-resistance element comprising a non-conductive body capable of reduction having a definite portion thereof reduced to an electrical conductive material and supported by said non-conductive body. 70

2. A high-resistance element comprising a chemical substance capable of reduction having a definite elongated portion thereof reduced to electrical conductive material. 75

3. A high-resistance element comprising a non-conductive oxide having a portion thereof reduced to electrical conductive material. 80

4. A high-resistance element comprising a body composed of a mixture of chemical substances capable of reduction and having a definite portion thereof reduced to electrical conductive material boarded by said substance. 85

5. A high-resistance element comprising a mixture of non-conductive oxides having a definite portion thereof reduced to electrical conductive material surrounded by said non-conductive oxides. 90

6. A high-resistance element comprising a body of chemical compounds capable of reduction and having a portion thereof of helical form reduced to provide an electrical conductor. 95

7. A high-resistance element comprising a body consisting of a mixture of non-conductive oxides having a portion thereof reduced to an electrical conductive material. 100

8. A high-resistance element comprising a continuous body of electrically conductive metal reduced from a supporting body consisting of the oxide of said metal. 105

9. A high-resistance element comprising a body of electrically conductive material reduced from, and embedded in, the surface 110 of a refractory oxide.

10. A high-resistance element comprising a body of a refractory oxide having a filamentary helical portion thereof reduced to provide an electrical conductor. 115

11. The method of forming a high-resistance conductor which consists in disposing upon a body of a chemical substance capable of reduction, a streak of material capable of reducing the said substance, heating the body and streak to effect a reducing action in the substance. 120

12. The method of forming a high-resistance conductor which consists in disposing upon a body of a non-conductive body capable of reduction, a filamentary material capable of reducing the body, heating the body and filament to effect a reducing action on the body. 125

13. The method of forming a high-resist- 130

ance conductor which consists in disposing about a body of a refractory oxide, a helical winding of a material capable of reducing said oxide, placing the body and winding thereon in an inert environment and heating the body and winding to effect a reducing action of the oxide adjacent said winding.

14. The method of forming a high-resist-  
10 ance conductor which consists in disposing about a body of thoria, a carbon strip, plac-  
ing the body in a furnace, heating to a re-

ducing temperature and finally removing the strip.

15. The method of forming a high-resist-  
15 ance conductor which consists in disposing about a body of thoria, a helically disposed carbon strip, placing the body in a furnace, heating to a reducing temperature and finally removing said strip.

In testimony whereof, I have hereunto  
subscribed my name this 16th day of March  
1923.

CHARLES FREDERICK LORENZ.